

## UNITED STATES PATENT OFFICE.

ALFRED EGGIMAN AND ALBINO PEREA, OF PARIS, FRANCE.

## COATING PROCESS.

No Drawing. Application filed December 1, 1924, Serial No. 753,342, and in France December 15, 1923.

This invention relates to a process for giving any article, for instance of wood, of metal, of cardboard or the like the appearance of enamel, porcelain, or natural or 5 artificial stone.

This process consists essentially in dipping the article successively and in any suitable order, into baths of determined composition, the article being more or less dried 10 between each dipping and receiving the colourings or powders which are intended to give it the desired appearance.

By the use of the process according to the invention any object manufactured in the 15 ordinary way from wood, metal, cardboard or from any other material can be given the appearance of enamel, mat or polished, of all tints or colourings, with or without rainbow effects, variegated or iridescent portions, the appearance of mother of pearl, of phosphorescence or of opal.

The objects may also be given the appearance of plain porcelain, which may be decorated, of majolica etc., or of burnt or fired 25 or other earthenware or of faience or other artificial products.

Moreover, according to the process forming the subject of the invention articles may be given the appearance of natural or artificial 30 stone which may be veined or not, such as lapis-lazuli, or the appearance of resins, amber or the like. Finally the process may be employed for imitating silvered, gilded, bronzed and like surfaces or for giving 35 spangled or diamond effects by the addition of powders or metal spangles of all tints and colours, natural or artificial crystals, transparent powdered glass, which may be clear or mat, the crystal or glass powder being 40 coloured or not.

The process forming the subject of the invention includes essentially the following stages or operations.

1. In the first place the article which may 45 be of any material formed to its definite shape, is covered with a preliminary coating by means of a paint brush or in any other manner, this preliminary coating being composed, in a known manner, from a mixture of linseed oil, turpentine and crushed white lead. The article is now allowed to dry, and after drying there is applied in the same manner a second coat similar to the first, and the article is again dried.

55 2. The object is then dipped into a bath

composed of two and a half litres of water, 60 500 grammes of gelatine and 500 grammes of zinc white, this bath being heated in a jacketed pan and kept at a temperature of about 40° to 45° centigrade.

3. After slightly drying, the article is then dipped into a bath composed of two and a half litres of water and 500 grammes of pure gelatine, kept at a temperature of about 40° to 45° centigrade to which colour is 65 added (aniline colour for instance) according to the tint of the foundation coat which may be desired, or the foundation coat may be white.

4. The article is then dipped into a bath 70 similar to the preceding, but not coloured; this bath only being coloured in the case where it is desired to obtain a foundation coat of deeper shade than those obtained by dipping in the preceding bath. The article 75 is again dried. Where it is desired to obtain a polished appearance, the following operations are also adopted.

5. The object is dipped into a collodion 80 bath and allowed to dry.

6. Finally it is dipped into a bath of varnish with a base of amyl acetate.

To give the object the appearance of porcelain or painted and decorated faience, the same operations are carried through, but a 85 thicker coating is applied in the bath containing gelatine and zinc white. The dipping in the bath of gelatine and colour is replaced by the application on the previous coating before it is completely dry, of alcohol colours, this application may be made by means of a sponge, by a vaporizing apparatus or by means of a paint brush, allowing the required decoration to be obtained (points, dabs, arabesques or the like 90 in one or more colours, which may be light or deep).

In the case in which it is desired to imitate natural or artificial stone, which may or may not be precious, between the dipping into the 100 bath of coloured gelatine and the dipping into the bath of pure gelatine, there is applied on the surface of the article, whilst still damp, a sponge slightly soaked in water and upon which has been shaken a certain amount of powder, either a metallic powder (bronze, silver, gold for example) or any coloured powder (for instance powdered glass or phosphorescent powder) or again spangles or crystals which may be 105 110

coloured or not, the powder being chosen suitably according to the stone which it is desired to imitate.

Lastly, in cases where instead of giving to 5 the article a polished surface, as described above, it is desired to give it a mat surface, for instance to imitate mat enamel with variegated effects, opal or mother of pearl, the operation described above under Nos. 5 and 10 6 respectively are replaced by the following:—

The article is dipped into a bath of colloidion with a cellulose acetate base, and after drying powder is applied for producing 15 the desired variegated effect, such powder being of any required description known in commerce. The powder is applied by means of a piece of buck skin and the object is finally dipped after this treatment into any 20 known liquid for producing a variegated or iridescent effect.

What we claim and desire to secure by Letters Patent of the United States of America is:—

- 25 1. A process for giving any object, of wood, metal, card or other material, the appearance of enamel, including the following operations, the application to the object of at least one preliminary coating of linseed oil, turpentine and crushed white lead, the drying of the object, and the dipping of the said object into at least one bath composed substantially in the proportions of 2½ litres of water, 500 grammes of gelatine and 500 grammes of zinc white, followed by the drying 30 of the object and the dipping thereof into a bath composed of about 2½ litres of water and 500 grammes of pure gelatine, substantially as described.
- 40 2. A process for giving any object, of wood, metal, card or other material, the appearance of enamel, including the following operations, the application to the object of at least one preliminary coating of linseed oil, turpentine and crushed white lead, the drying of the object, the dipping of the said 45

object into at least one bath composed substantially in the proportions of 2½ litres of water, 500 grammes of gelatine and 500 grammes of zinc white, the dipping of the 50 said object into a bath composed of about 2½ litres of water and 500 grammes of pure gelatine, to which colour is added according to the tint required, substantially as described. 55

3. A process for giving any object, of wood, metal, card or other material, the appearance of enamel, including the following operations, the application to the object of at least one preliminary coating of linseed oil, 60 turpentine and crushed white lead, the drying of the object, the dipping of the said object into at least one bath composed substantially in the proportions of 2½ litres of water, 500 grammes of gelatine and 500 grammes of zinc white, drying the said object, dipping the said object into a bath composed of about 2½ litres of water and 500 grammes of pure gelatine, dipping the object into a collodion bath, allowing the same 65 to dry and finally dipping it into a bath of varnish with a base of amyl acetate. 70

4. A process for giving any object, of wood, metal, card or other material, the appearance of enamel, including the following 75 operations, the application to the object of at least one preliminary coating of linseed oil, turpentine and crushed white lead, the drying of the object, the dipping of the said object into at least one bath composed of gelatine zinc white mixed with water, 80 drying the said object, dipping the said object into a bath of pure gelatine dissolved in water, drying the said object and dipping the same into a varnishing bath with 85 a base of amyl acetate, substantially as described.

In witness whereof we have hereunto affixed our signatures.

ALFRED EGGIMAN.  
ALBINO PEREA.